

# UNITED STATES PATENT OFFICE.

JAMES H. DANVER, OF BEAVER, PENNSYLVANIA, ASSIGNOR TO UNITED STATES SANITARY MANUFACTURING COMPANY, OF PITTSBURG, PENNSYLVANIA, A CORPORATION OF PENNSYLVANIA.

## METHOD OF MAKING MOTTLED ENAMEL.

1,001,511.

Specification of Letters Patent. Patented Aug. 22, 1911.

No Drawing.

Application filed November 30, 1909. Serial No. 530,683.

To all whom it may concern:

Be it known that I, JAMES H. DANVER, of Beaver, Beaver county, Pennsylvania, have invented a new and useful Method of Making Mottled Enamel, of which the following is a full, clear, and exact description.

My invention relates to providing metallic articles, such as sinks, laundry tubs, &c., with a mottled enamel surface, and is designed to give a more attractive appearance to the article than that heretofore imparted by processes for applying mottled enamel.

In carrying out my invention, I prepare the coloring material in two or more different batches. Each batch is made up by mixing glass cullet (preferably clear or crystal glass) with the coloring material, which preferably consists of a metallic oxid or oxids. The glass forms the larger portion of the mix, and is preferably in proportion of about 90 to 95 per cent., the remainder consisting of the coloring material such as metallic oxid. The glass of each batch thus made up is then fused so as to disseminate the coloring material throughout the glass body or carrier. The oxid for one batch is preferably of one color, such as blue, while the other oxid for the other batch is preferably of another color, such as brown or red. The two fused batches of glass of different colors are then separately ground up, preferably to a slightly larger size than that of the white or lighter colored enamel with which they are mixed.

The use of two different colors gives a stronger and more pronounced appearance than with former processes. The shade or tint may also be varied by varying the proportions of the two coloring materials. If the coloring materials of different colors were fused in the same glass batch, the tint or shade could not be varied and a dead appearance would be imparted. Furthermore, a more uniform effect can be obtained, since in the use of a single mix of the coloring material the particular degree of heat applied will vary the intensity of the color to some extent, and hence, where the same proportions of the final mix are used, the tint or color will be darkened or made lighter with different batches. This can be corrected by the use of the two different

color batches—by increasing or decreasing 55 the percentage of one of the coloring ingredients.

After the two or more colored glass batches have been made and ground up they are mixed in the usual way and in the desired proportions with ground-up white enamel, which latter has been ground preferably to a greater degree of fineness than the colored batches. The three or more mixed materials are then sifted upon the metallic surfaces, which is preferably pre-heated. The article is then heated to the ordinary temperature for fusing the white enamel. A base coat may be used on the article before the mottling coat of enamel 70 is applied, and two or more mottling coats may be applied successively.

The advantages of my invention result from the use of glass as a carrier for the color ingredients, and also from the use of 75 two or more batches of coloring materials of different colors.

Within my broader claims covering the use of different colors, the colored material may be glass or enamel; and many other 80 changes may be made in the process without departing from my invention.

I claim:

1. In the method of making mottled or colored enamel, the steps consisting of mixing coloring material with glass, fusing the same, comminuting the resulting colored glass, and mixing this comminuted material with a differently colored enamel, substantially as described. 90

2. In the method of making mottled or colored enamel, the steps consisting of mixing metallic oxid with glass, fusing the same, comminuting the resulting colored glass, and then mixing the comminuted colored glass with enamel of a lighter color, substantially as described. 95

3. In the method of making mottled or colored enamel, the steps consisting of separately fusing two or more batches of coloring material of different colors, grinding the same and mixing the different colors with a white or relatively lighter enamel; substantially as described. 100

4. In the method of making mottled or colored enamel, the steps consisting of fusing two or more portions of coloring material of different colors with different batches 105

of glass, fusing the same separately; grinding the resulting materials separately and mixing two or more of said coloring materials with white or relatively lighter enamel; 5 substantially as described.

5. In the method of making mottled or colored enamel, the steps consisting of mixing coloring material with glass, fusing the same, comminuting the resulting colored 10 glass, and mixing this colored glass while

in a dry comminuted form with a comminuted differently colored dry enamel, substantially as described.

In testimony whereof, I have hereunto set my hand.

JAMES H. DANVER.

Witnesses:

C. P. BYRNES,  
H. M. CORWIN.